

# United States Patent Office

2,880,085

Patented Mar. 31, 1959

1

2,880,085

## FERRITIC ALLOY STEELS FOR USE AT ELEVATED TEMPERATURES

Henry William Kirkby and Charles Sykes, Sheffield, England, assignors to Firth-Vickers Stainless Steels Limited, Sheffield, England, a British company

No Drawing. Application March 11, 1957  
Serial No. 645,004

Claims priority, application Great Britain March 29, 1956

5 Claims. (Cl. 75—126)

This invention relates to improvements relating to ferritic alloy steels for use at elevated temperatures.

An object of the invention is to provide a forgeable ferritic alloy steel possessing improved creep resistance at temperatures up to 700° C.

British specification No. 658,115 (hereinafter referred to as the earlier specification) describes a forgeable ferritic alloy steel having a composition characterised by the absence of nickel above a proportion of 1.5% and by the presence as essential constituents of 0.05—0.5% carbon, 4—20% chromium, 0.5—3% molybdenum and/or tungsten, 0.2—2.5% niobium, 0.05—0.25% nitrogen, 0.003—0.5% boron and 0.1—2% vanadium. The alloy may also contain silicon up to 3%, manganese up to 4% and cobalt up to 10%.

The preferred proportions of the various constituents, as described in the earlier specification are:

|                                                | Percent       |
|------------------------------------------------|---------------|
| Carbon                                         | 0.10 to 0.25  |
| Silicon                                        | 0.5 to 1.5    |
| Manganese                                      | 0.5 to 1.5    |
| Nickel                                         | 0.5 to 1.5    |
| Chromium                                       | 10.0 to 14.0  |
| Molybdenum and/or                              | 0.5 to 1.5    |
| Tungsten (The maximum total content being 3%). | 1.0 to 3.0    |
| Vanadium                                       | 0.1 to 0.3    |
| Niobium                                        | 0.5 to 1.25   |
| Nitrogen                                       | 0.10 to 0.15  |
| Boron                                          | 0.025 to 0.10 |
| Cobalt                                         | Nil to 5.0    |
| Iron                                           | Remainder     |

Alloy steels of the above composition possess stress-to-rupture properties of the following order:

| At 650° C.:     | Rupture strength (hrs.) |
|-----------------|-------------------------|
| 15 tons/sq. in. | 463                     |
| 17 tons/sq. in. | 30                      |

It has now been found that with certain modification in the composition described in the earlier specification substantially higher rupture strength at 650° C. can be obtained. It will be noted that in the earlier composition the maximum range of the tungsten content was 0.5 to 3.0%. According to the principal modification of the present invention an increased amount of tungsten is incorporated, the new range being over 3% and up to 16%.

The alloys of this invention comprise as essential constituents 0.03 to 0.30% carbon, 4% to 20% chromium, over 3 and up to 16% tungsten, 0.1 to 2.0% vanadium, and 0.05 to 2.5% niobium interchangeable wholly or in part by tantalum. The alloys may also contain up to 2.0% silicon, up to 4% manganese, up to 1.5% nickel, up to 0.25% nitrogen, up to 0.5% boron and up to 20% cobalt.

2

The preferred proportions of the various constituents are as follows:

|                                         | Percent             |
|-----------------------------------------|---------------------|
| Carbon                                  | 0.03 to 0.20        |
| Silicon                                 | 0.3 to 1.5          |
| Manganese                               | 0.5 to 1.5          |
| Nickel                                  | 0.1 to 1.0          |
| Chromium                                | 9.0 to 16.0         |
| Tungsten                                | Over 3.0 up to 10.0 |
| Vanadium                                | 0.1 to 0.7          |
| Niobium (interchangeable with tantalum) | 0.05 to 1.0         |
| Nitrogen                                | Up to 0.10          |
| Boron                                   | Up to 0.10          |
| Cobalt                                  | 5.0 to 15.0         |
| Iron                                    | Remainder           |

In the above alloys molybdenum up to 3% may be added, in which case it replaces a corresponding proportion of the iron remainder.

After suitable heat treatment, typical alloys (identified as alloys A, B, C, respectively) within the invention possess (as compared with the alloys of the earlier specification) the following properties, expressed as the stress for the 100 hours rupture strength at 650° C.:

| 25 | Earlier Specification       | Alloy A, tons/sq. in. | Alloy B, tons/sq. in. | Alloy C, tons/sq. in. |
|----|-----------------------------|-----------------------|-----------------------|-----------------------|
| 30 | 16-16½ tons/sq. in. approx. | 20                    | 25                    | 28                    |

The alloys A, B, C contain respectively 4%, 6% and 8% of tungsten, and it will be noted that, with the particular alloys concerned, the rupture strength is approximately a function of the tungsten content.

35 As is known, the creep resistance of an alloy steel depends to some extent on the heat treatment to which it has been subjected. The term "suitable heat treatment" as used above is intended to convey that the temperature, the rate of heating and cooling, and the duration of the treatment are such that optimum properties are developed for the particular composition. An example of heat treatment suitable in some cases is to harden in air or oil from about 1160° C. followed by a tempering treatment at 675° C.

45 We claim:

1. A forgeable ferritic alloy steel comprising 0.03 to 0.30% carbon, 4 to 20% chromium, over 3 and up to 16% tungsten, 0.1 to 2.0% vanadium, and 0.05 to 2.5% of at least one element from the group consisting of niobium and tantalum, and the balance iron with incidental impurities in ordinary amounts.

50 2. A forgeable ferritic alloy steel comprising, 0.03 to 0.30% carbon, 4 to 20% chromium, over 3 and up to 16% tungsten, 0.1 to 2.0% vanadium, up to 2% of silicon, up to 4% of manganese, up to 1.5% of nickel, up to 0.25% nitrogen, up to 0.5% of boron, up to 20% of cobalt, 0.05 to 2.5% of at least one element from the group consisting of niobium and tantalum, and the balance iron with incidental impurities in ordinary amounts.

60 3. A forgeable ferritic alloy steel comprising, 0.03 to 0.20% carbon, 0.3 to 1.5% silicon, 0.5 to 1.5% manganese, 0.1 to 1.0% nickel, 9 to 16% chromium, over 3 and up to 10% tungsten, 0.1 to 0.7% vanadium, 5 to 15% cobalt, up to 0.10% nitrogen, up to 0.10% boron and 0.05 to 1.0% of at least one element from the group consisting of niobium and tantalum, and the balance iron with incidental impurities in ordinary amounts.

70 4. A forgeable ferritic alloy steel comprising, 0.03 to 0.30% carbon, 4 to 20% chromium, over 3 and up to 16% tungsten, 0.1 to 2.0% vanadium, up to 2.0% of silicon, up to 4.0% manganese, up to 1.5% of nickel,

up to 0.25% of nitrogen, up to 0.5% of boron, up to 20% of cobalt, up to 3% of molybdenum, and 0.05 to 2.5% of at least one element from the group consisting of niobium and tantalum, and the balance iron with incidental impurities in ordinary amounts.

5. A forgeable ferritic alloy steel article characterized by a rupture strength, expressed as stress for 100 hours at 650° C. of the order of 20 to 28 tons per square inch and having a composition consisting essentially of nickel up to about 1.5%, of 0.03 to 0.30% carbon, 4 to 20% chromium, 4 to 8% tungsten, 0.1 to 2.0% vanadium and 0.05 to 2.5% of at least one element selected from the

group consisting of niobium and tantalum, and the balance iron with incidental impurities in ordinary amounts.

References Cited in the file of this patent

UNITED STATES PATENTS

|           |               |               |
|-----------|---------------|---------------|
| 2,253,385 | Mahin         | Aug. 19, 1941 |
| 2,432,614 | Franks et al. | Dec. 16, 1947 |
| 2,462,665 | Olcott        | Feb. 22, 1949 |
| 2,542,220 | Urban et al.  | Feb. 20, 1951 |
| 2,590,835 | Kirkby et al. | Apr. 1, 1952  |